

## UNITED STATES PATENT OFFICE

2,409,818

## BRUSH AND ART OF COMMUTATION

Hugh H. Wikle, Cleveland Heights, Ohio, assignor to Superior Carbon Products, Inc., Cleveland, Ohio, a corporation of Ohio

No Drawing. Application November 4, 1942,  
Serial No. 464,531

11 Claims. (Cl. 171—325)

1

This invention relates to brushes for dynamoelectric machines, more particularly those of the so-called carbon or graphite type, to a method of making such brushes and a method and means of improving brush life, commutation and brush operation.

In the art to which this invention relates the problem of excessive brush wear on electric machines, as for example in airplanes around and above 20,000 feet of altitude, has long defied solution. Particularly in the exigency of war, this problem has become increasingly critical. Other problems have been concurrently present, at both low and high altitudes, in form of relatively high friction between the brushes and commutators and slip rings, relatively high specific resistance in the body of the brush, relatively low current density and relatively low contact resistance. Factors of economy and facility of manufacture have been preserved and enhanced in my solution of these problems.

It is among the objects of my invention to provide a brush which will have long and satisfactory life in service at high altitudes, particularly altitudes in excess of 20,000 feet. Another object is to provide a brush capable of performing satisfactorily with a high current density without physical or electric deterioration or excessive sparking under a wide range of operating conditions including extreme conditions of altitude and temperature. A further object is to provide a brush, which in its use in dynamoelectric machines, as in contact with commutators and slip rings, will perform satisfactorily through a wide range of conditions with less frictional loss than prior art brushes. Another object is to provide a brush retaining or improving its characteristics of contact resistance while carrying out my other objects. A further object of my invention is to provide a brush which will achieve the foregoing objects without sacrifice of physical strength, or with relatively increased physical strength. Another object is to provide an economical and facile method of making such brushes. Another object is to provide an improved method of commutation and an improved method of brush operation in respect to wear, friction, contact resistance, sparking and the like. These and other objects of my invention will become more fully apparent in the following description of a preferred and certain modified forms of my invention. The essential characteristics are summarized in the claims.

While I do not care to be committed to any particular philosophical speculation as to the

2

why or the wherefore of the manner in which my brushes or methods work and obtain their results, still I have made some observations and drawn some tentative conclusions which I believe will be helpful to those skilled in the art in their understanding and practice of my invention. I mention and refer to these things without prejudice as to the metes and bounds of my invention or patent claims. I believe that in the ordinary use of the prior art brushes at or around sea level and in the ordinary range of temperatures in which dynamoelectric machines with brushes have been commonly used that the successful operation of the brush is coincident with the formation of or the deposition of a thin or microscopically thin film or coating on the commutator or slip ring and perhaps also on the adjacent face of the brush. I believe that under these known prior art conditions this film comprised largely cupreous or cupric oxide, particles of carbon or graphite and other constituents of the brush, impurities such as grease and dirt and perhaps also oxygen, water vapor and other atmospheric gases. Whatever the constituents of such a film, it seems to have had the function of reducing friction between the brush and commutator or slip ring, aiding in the maintainence of contact resistance and otherwise performing such a beneficent purpose that upon its substantial impairment or elimination, mechanical wear and abrasion increase very rapidly, contact resistance is lowered with accompanying electric disturbances such as sparking, and other evidences of poor commutation appear. It appears to me that the presence of oxygen and water vapor aid in or give facility to the formation of such film as I have described or at least that their presence is consistent with conditions under which such a film seems to exist. I have observed that during attempted brush operation in an atmosphere of dry nitrogen the brush wear and abrasion increases noticeably and other undesirable conditions of commutation quickly appear.

One of the recognizable conditions at high altitude with the accompanying low temperature is the relative lack of oxygen and water vapor, and I believe that this deficiency may have much to do with the rapid and dangerous brush wear under this condition. My thought has been to provide a film or the equivalent in respect to the functions which I believe have been performed by the film above described, and which would not be dependent upon, among other things, the relatively abundant presence of oxygen and

water vapor or the conditions obtaining therein. I have found that my improvement in this particular respect has been accompanied by other improvements of broad and general benefit.

Regardless of the accuracy of my philosophical premises and assumptions, I have found that by adding sulphur to the constituents of a graphite brush in a manner which I believe preserves the sulphur at least in part in the form of free sulphur or in a form whether free or compounded that is reactive with or adherent to the copper of the commutator or slip ring, that my desired results are obtained. By making sulphur available to and at the brush and commutator or slip ring and/or incorporating it in the brush in the manner about to be described I have been able to achieve the objects of my invention.

I am aware on the one hand that the presence of relatively small amounts of sulphur in one form or another in prior art carbon brushes has been thought to be deleterious and effort has been made to eliminate it. I am also aware that relatively large quantities of sulphur have been included in the mix in the making of other types of prior art carbon brushes, but that in both instances the advantages which I have sought to obtain have been lost. I believe that the disadvantage commonly recognized in the presence of a small amount of sulphur and the absence of advantage in the prior practice of endeavoring to use large quantities of sulphur are wholly or partly due to using either or all carbon flour and pitch binders with the sulphur and subjecting such brushes to such high temperatures during the baking thereof as to boil away or vaporize the sulphur or sulphur compounds or so combine the sulphur with other constituents of the brush as to inhibit the function and results which I have been able to obtain.

A specific example of a preferred form of the composition of and a preferred method of making brushes embodying or made in accordance with my invention is: Two gallons of shellac are mixed with 42 pounds of Ceylon graphite, the shellac having the consistency commercially known as  $4\frac{1}{2}$  pound, meaning it contains about  $4\frac{1}{2}$  pounds of resin or solid material to every gallon of solution including volatile solvents. The mixture above described is mechanically mixed until substantially all parts of the graphite are "wetted" with the shellac solution albeit the proportion of shellac to graphite is such that the so-called wetness is not clearly apparent to the eye. After a thorough mixture of these constituents the mixture is permitted to dry at room temperature preferably being spread out in a relatively thin layer in appropriate drying pans until substantially all the volatile solvents of the shellac solution that will evaporate at room temperatures have passed off. When this mixture has been dried to this extent I take 18 pounds of mixture and add preferably 2 pounds of dry powdered sulphur. These ingredients are thoroughly mixed mechanically at room temperature and then pressed, preferably in the form of a block about 5 to 6 inches square and about  $\frac{1}{4}$  to  $1\frac{1}{2}$  inches deep, depending on the thickness desired in the finished brushes, under a gross pressure of about 200 tons, i. e., at about 6 to 7 tons per square inch. This block of brush material, from which the brushes of appropriate size and shape may subsequently be cut, is then heated slowly and gradually brought up to a temperature of about 500° Fahrenheit and held at about that temperature for a period of about

48 hours. After cooling the baked and molded mass will be found to be firmly bonded in a solid block, and will have satisfactory physical characteristics to facilitate its severance into desired sizes and shapes for brush use. I prefer, for reasons known to those skilled in the art, to control the thickness of the block, i. e., its depth in the direction of application of molding pressure, and then cut or sever the block into sizes and shapes of finished brushes in such a way that when the brush is placed in operative relation to the commutator, the direction of application of molding pressure will lie substantially tangentially of the commutator.

Brushes made in the preferred form and by the preferred steps described above have given satisfactory long life under high altitude conditions. Moreover, the brushes embodying my invention have shown ability to carry current densities of the order of about 175 amperes per square inch as compared with current densities of the order of 60 amperes per square inch in similar prior art brushes lacking the sulphur constituent. I have also observed that brushes embodying my invention in its preferred form have as little as about one-half the specific resistance of such prior art brushes while retaining a high or improved contact resistance. Moreover, the brushes embodying my invention reduce the friction loss between the brush and commutator or slip ring up to about one-half and do all these things without sparking or physical or electric disintegration or deterioration and without sacrifice of physical strength under the ordinary and normal conditions of use as well as under the extreme conditions of high altitude airplane operation above about 20,000 feet.

In the operation of brushes containing my invention I have observed that at the beginning of use on a clean commutator there appears to be formed on the commutator a dull chocolate colored polish or film which, as such, seems to disappear under sea level conditions of use after about 8 to 10 hours operation. And, I have observed that if thereafter the commutator be sanded and again cleaned and the machine run again, the so-called film or polish reappears and again remains visible for about 8 to 10 hours of such operation. From these observations a theory of operation suggests itself, which I advance without prejudice, (1) that under sea level conditions the said visible film or polish is supplied by the sulphur, and/or sulphur and binder or other mixtures or compounds including sulphur, which was contained in the initially exposed bearing surface of the brush, and that the remaining constituents of the exposed surface wore so slowly under those sea level conditions, that the ingredients of the visible sulphur bearing film were not exposed or released from within the brush at a rate rapid enough to be visible, after their initial appearance and 8 to 10 hours wear. (2) Under high altitude conditions the increased tendency to wear away the bearing surface of the brush removes the non-film forming constituents in the face of the brush thus exposing an additional increment of film forming ingredients which in turn retard or tend to eliminate the wear. A balance is thus provided in which the very wear of the brush face, instead of beginning a cycle of self-destruction as in the prior art practice, constitutes the means of self-preservation within the precepts of my invention. My observations of tests performed with my brush under or simulating high altitude conditions evi-

dence that the life of the brush containing the proportion of parts in the preferred example given above is extended about a hundred fold more or less the life of prior art brushes.

In the practice of my invention I contemplate the admixture of sulphur in amounts varying substantially from the precise proportion above described without departing from the precepts of my invention, and I contemplate the use of compounds and mixtures of sulphur as well as commercially powdered chemically pure sulphur so long as the change of proportion and the nature of the mixture of compounds do not substantially defeat the essential function and contribution to the mode of operation of my invention that is performed by the sulphur or its compounds, mixture or equivalents in the preferred example above given. Although I have indicated a preference for a 10% mixture of sulphur with the other constituents of my brush, I have varied the proportion from about 5% to 15% sulphur with satisfactory results. I mention these variations by way of example rather than limitation. Those skilled in the art may be guided in the same or different changes in proportions within the precepts of my invention, having in mind that brush life at high altitudes tends to be increased, as I believe for the reasons given above, with the larger proportions of sulphur, although under some conditions of use I expect that further increases in the proportion of sulphur in a brush otherwise following my preferred form will tend to restrict its utility in point of physical strength. Again, I have observed within limited test conditions that while my brush having 5% to 10% sulphur substantially halves the specific resistance, compared with similar brushes lacking any sulphur, my brush with 15% sulphur tends to show some increase in specific resistance on the same comparison. Again, while my brush having 5% to 10% sulphur appears to substantially equal the non-sulphur prior art brush in point of contact resistance, my brush with 15% sulphur has tended to show about one-third increase in contact resistance by the same comparison.

While I have employed shellac for a binder in the preferred form above mentioned I do not mean to exclude other chemically and/or mechanically equivalent binders. For guidance rather than limitation I mention a few of the characteristics and functions of the binder that I prefer. It performs its binding function, i. e., is cured and sets, at low temperatures in relation to the vaporization or boiling point of sulphur so that sulphur is not driven from the mix during the baking step. It holds the sulphur in the finished brush whether mechanically or chemically or both in such a way that at least under the conditions of commutation a reaction between part of the sulphur and the metal of the commutator is not substantially impaired or inhibited. Preferably also it serves as a vehicle to carry the sulphur from the brush to the commutator or ring and tends to hold it in the film thereon; the binder thus also preferably entering into the contents of the film and giving it adhesion to the commutator. It also appears that the binder should not, in the form it takes on the commutator or wearing surface of the brush, be abrasive nor substantially diminish the "lubricating" effect of the film.

Even at the temperature of 500° Fahrenheit that I have mentioned in the preferred form of my invention for baking or curing my product I believe there is a loss of about 10 to 15% of the

sulphur from the original mix and I suggest that this tendency to loss be kept in mind particularly where smaller percentages of sulphur and/or higher baking temperatures are sought to be employed than I have suggested in my preferred example.

Although I have specified the use of Ceylon graphite as a preferred form of carbon or conducting element of the brush containing my invention my preference is to use graphite in the so-called flake or crystalline form. I prefer to use graphite as the carbon element of the brush especially where shellac is employed as the binder, because I believe the absorbent or adsorbent characteristic of carbon flour for example, tends to impair the binding function of the shellac. I do not exclude from my teaching the use of carbon in forms other than the form of graphite especially where binders that have the other characteristics which I desire are available and are not subject to substantial impairment in their desired function by association with other such forms of carbon.

While I have indicated a preference for drying the mixture of shellac, volatile solvents and graphite at room temperatures, and have found this practice most satisfactory and economical, I do not insist that this drying may not be expedited advantageously with other well known means or methods for drying comparable mixtures, such as drying under vacuum.

My inventive thought also takes the form and expression of a method of commutation in the steps of bringing sulphur to or between the wearing surfaces of brush and commutator or slip ring in a form and under conditions in which it will participate or aid in forming a wear resisting or lubricating film such as described above. Although as indicated I prefer to practice this method by the employment of my preferred form of brush participating in the electrical operation of the machine, I do not exclude other ways or means of forming the sulphur bearing film between brush and commutator. For example a separate or "third brush," within or without the electrical circuit, can be provided to bear on the commutator or ring in its wearing zone and can comprise sulphur and preferably a vehicle therefor such as shellac and preferably also some graphite particularly if the electrically active brushes lack these latter ingredients.

By way of further example of a practice of a form of my invention emphasizing the latter precepts, I have impregnated carbon brushes with sulphur and/or with sulphur and shellac or other resinous substances, and in the use of such brushes obtained a film having the desirable characteristics mentioned above. Such brushes retain substantially their normal internal electrical characteristics with increased contact resistance and reduced friction between brush and commutator and improved wear resisting characteristics.

In this practice of my invention I first form the carbon, carbon graphite, or carbon metal graphite brushes in the usual way as with pitch binder, compression molding and relatively high temperatures baking, employing carbon flour in the first instance and mixtures of carbon flour and graphite, or powdered metal or both as may be desired to give the known characteristics of brushes inherent in these mixtures and well known processes of manufacture. For my illustrative purpose such brushes are known to have certain

porosity and absorptive or adsorptive qualities conducive to impregnation by additional constituents.

I have found that such a carbon brush or a molded and cured block of such brush material in a slab 10" x 6" x 1/2" when immersed in sulphur in the liquid state at a temperature of about 250° F. at about 90 pounds pressure above atmospheric pressure for a period of about one hour will cause the brush or brush material to be impregnated with sulphur to the extent of about 30% of its total mass by weight, such pressure being conveniently maintained pneumatically over the bath. Thicker brushes or block will require this treatment for a longer period of time or at higher pressures, and thinner brushes or block will correspondingly require less time and pressure for the same extent of impregnation. Similarly when less impregnation is sought, lower pressures for shorter periods will provide a convenient means for regulating the extent of impregnation and correspondingly reduce the proportion of sulphur absorbed by the brush. Instead of using sulphur in the hot liquid state I may also impregnate similar brushes with colloidal sulphur carried by suitable vehicles such as mineral oil, alcohol or animal fats which can be driven off or will evaporate at appropriately mild temperatures, leaving the sulphur deposited within the interstices of the brush structure. With colloidal sulphur, impregnation can take place at room temperature with pressure applied to the bath in which the brush is immersed for a suitable length of time within the precepts mentioned above. Those understanding the art of impregnating such materials will also understand that the process may be hastened by first evacuating the air from the interstices of the brush or block of brush material about to be impregnated.

It may on occasion be desirable to first impregnate with a surplus of sulphur and thereafter reduce the sulphur content by baking the brush at temperatures varying from 500° to 1000° F. and by volatilizing or boiling off the excess sulphur. The time of such baking and the temperature will be controlled in relation to the extent to which it is desired to drive off the excess sulphur. By this means, the percentage of sulphur in the brush may be conveniently modified and controlled.

Within the practice of my invention involving the impregnation of carbon brushes with sulphur as above described, I also prefer to impregnate such brushes with resinous material such as shellac, which as mentioned in the preceding part of this specification seems to contribute to the formation and function of the film on the commutator. Such additional impregnation can be carried out by merely soaking the brush or block of brush material in a shellac solution such as the 4 1/2 pound solution first above described for a matter of a few hours at room temperature and pressure. The volatile solvents of the shellac solution will pass out of the brush in a relatively short time at ordinary room temperatures or may be driven off with mild heat- 65

Within the teaching of the foregoing example I do not mean to exclude repetitive steps of impregnation at pressures and times differing substantially from those mentioned above. Neither do I exclude combining the steps of impregnating with sulphur and impregnating with shellac or other resins where that may be found advantageous or expedient. For example where a common vehicle or solvent or mixture thereof will carry both shellac and colloidal sulphur they may both be forced into the interstices in one operation or a series of operations involving both the sulphur and shellac.

While I have described a preferred and certain modified forms of my invention in the brush as an article and the combination of a brush with a commutator or slip ring and in respect to my method inventions allied thereto, I do not care to be limited to the example disclosed herein or in any manner other than by the claims hereof.

I claim:

1. A brush comprising graphite, shellac and about 5% to 15% sulphur.
2. A brush comprising graphite, shellac and about 5% to 10% sulphur, and having only about half the specific resistance of a similar brush lacking sulphur.
3. A brush comprising graphite, shellac and sulphur in substantially the proportion of 42, 9 and 3 to 9 parts respectively.
4. The method of making brushes which consists in forming a mechanical mixture of graphite, sulphur and shellac, pressing the constituents into a substantially solid mass and baking the mass at a temperature of about 500° F. for about 48 hours.
5. The method of making brushes which consists in forming a mechanical mixture of graphite, sulphur and a binder, pressing the constituents into a substantially solid mass, warming the mass slowly to a temperature of about 500° F. and baking the mass at about such temperature for about 48 hours.
6. The method of making carbon brushes which consists in mixing carbon in one of its forms which conducts electricity, a binder capable of taking its set or cure at a temperature lower than the volatilizing temperature of sulphur, and sulphur, mixing such ingredients, and compressing and curing the same without raising the temperature substantially above 500° F.
7. A brush comprising carbon, a binder and about 5% to 15% sulphur.
8. A brush comprising graphite, a binder and about 5% to 15% sulphur.
9. A carbon brush impregnated with from about 5% to 30% sulphur.
10. A carbon brush impregnated with a binder and from about 5% to 30% sulphur.
11. A carbon brush impregnated with shellac and from about 5% to 30% sulphur.

HUGH H. WIKLE.